



US005401623A

**United States Patent** [19]**Texter**[11] **Patent Number:** **5,401,623**[45] **Date of Patent:** **Mar. 28, 1995**

[54] **REACTIVITY CONTROL IN  
MICROCRYSTALLINE COUPLER  
DISPERSIONS**

5,110,717 5/1992 Czekai et al. .... 430/512  
5,223,385 6/1993 Hasebe ..... 430/546  
5,240,821 8/1993 Texter et al. .... 430/546

[75] **Inventor:** **John Texter, Rochester, N.Y.**

**FOREIGN PATENT DOCUMENTS**

[73] **Assignee:** **Eastman Kodak Company,  
Rochester, N.Y.**

1105761 7/1981 Canada .  
0138831 11/1979 Germany .  
0139040 12/1979 Germany .  
236603 6/1986 Germany .  
1193349 5/1970 United Kingdom .  
1570362 7/1980 United Kingdom .

[21] **Appl. No.:** **956,140**

[22] **Filed:** **Oct. 5, 1992**

[51] **Int. Cl.<sup>6</sup>** ..... **G03C 1/08; G03C 7/26;  
G03C 7/32**

[52] **U.S. Cl.** ..... **430/546; 430/377;  
430/543**

[58] **Field of Search** ..... **430/546, 449, 377, 543,  
430/464, 470**

*Primary Examiner*—Charles L. Bowers, Jr.  
*Assistant Examiner*—Geraldine Letscher  
*Attorney, Agent, or Firm*—Paul A. Leipold

[56] **References Cited**

**U.S. PATENT DOCUMENTS**

2,870,012 1/1959 Godowsky et al. .... 430/546  
3,676,147 7/1972 Boyer et al. .... 430/569  
4,006,025 2/1977 Swank et al. .... 430/567  
4,474,872 10/1984 Onishi et al. .... 430/512  
4,490,461 12/1984 Webb et al. .... 430/510  
4,927,744 5/1990 Henzel et al. .... 430/566  
4,948,718 8/1990 Factor et al. .... 430/522  
4,970,139 11/1990 Bagchi .... 430/449  
5,008,179 4/1991 Chari et al. .... 430/546  
5,089,380 2/1992 Bagchi .... 430/449

[57] **ABSTRACT**

A photographic coupler dispersion comprising colloidal microcrystalline particles of coupler, wherein said particles are wetted with an activating and water-immiscible organic solvent, and a color photographic element comprising a support bearing at least one photographic silver halide emulsion layer and a microcrystalline coupler dispersion in reactive association with said emulsion layer, wherein said coupler is wetted with an activating water-immiscible organic solvent are disclosed.

**15 Claims, 13 Drawing Sheets**

**FIG. 1****FIG. 2**

FIG. 3



FIG. 4



FIG. 5



FIG. 6



FIG. 7



FIG. 8



FIG. 9



FIG. 10



FIG. 11



FIG. 12



FIG. 13



FIG. 14



FIG. 15



FIG. 16



FIG. 17



FIG. 18



FIG. 19



FIG. 20



FIG. 21



FIG. 22



FIG. 23



REACTIVITY CONTROL IN  
MICROCRYSTALLINE COUPLER DISPERSIONS

FIELD OF THE INVENTION

This invention relates to photographic systems and processes for forming image dye in light sensitive silver halide emulsion layers and to the nature of the photographically active coupler dispersions used to form said dye image. More particularly this invention relates to the composition and morphology of said coupler dispersions, the physical state of coupler in said dispersions, and the reactive association of said coupler molecules with activating water-immiscible organic solvents.

BACKGROUND OF THE INVENTION

Godowsky and Duane, in U.S. Pat. No. 2,870,012, disclose a solvent-shifting process for preparing micro-dispersions of color coupler compounds comprising at least one acid group (carboxyl or sulfonic acid).

Townsley and Trunley, in U.K. Pat. No. 1,193,349, disclose a solvent-shifting and pH-shifting process in the presence of a protective colloid for dispersing couplers as amorphous colloidal dispersions. Their process is applied to couplers that have no sulphonic acid or carboxylic acid solubilizing groups and that are soluble in a mixture of water-miscible organic solvent and aqueous alkali.

Webb et al. in U.S. Pat. No. 4,490,461, disclose a process for the preparation of a photographic material comprising at least one silver halide emulsion layer and which contains in at least one layer a photographically useful compound selected from the group consisting of developing agents, color couplers, optical brighteners, filter dyes, or acutance dyes. Said process comprises forming a solution of a photographically useful compound, a compound capable of being cross-linked, and a cross-linking agent for the cross-linkable compound, effecting cross-linking of the cross-linkable compound to form a cross-linked solid, isolating the solid and milling the solid to form particles of 0.1-0.5  $\mu\text{m}$  in size, dispersing the particles in a colloid binder coating solution, coating this solution on a photobase and drying the layer.

Bagchi, in U.S. Pat. Nos. 4,970,139 and 5,089,380, discloses methods of preparing precipitated coupler dispersion with increased photographic activity. Said methods comprise steps to simultaneously precipitate hydrophobic couplers in the form of small particles and wherein said particles incorporate at their instant of formation water-insoluble coupler solvents.

Chari et al., in U.S. Pat. No. 5,008,179, disclose the preparation of amorphous coupler dispersions by pH and solvent shifting and the mixing of said coupler dispersions with dispersions of permanent solvent immediately prior to preparing light sensitive coating melts. This process of combining permanent solvent with amorphous coupler dispersion minimizes certain difficulties arising from crystallization of said coupler during storage of the coupler dispersion. Chad et al. disclose the preparation of permanent solvent dispersions wherein the permanent solvent is loaded into a polymeric latex.

Langen et al., in U.K. Pat. No. 1,570,362 disclose the use of solid particle milling methods such as sand milling, bead milling, dyno milling, and related media, ball, and roller milling methods for the production of solid particle dispersions of photographic additives such as

couplers, UV-absorbers, UV stabilizers, white toners, stabilizers, and sensitizing dyes.

Henzel and Zengerle, in U.S. Pat. No. 4,927,744, disclose photographic elements comprising solid particle dispersions of oxidized developer scavengers. Said dispersions are prepared by precipitation and by milling techniques such as ball-milling.

Boyer and Caddi, in U.S. Pat. No. 3,676,147, disclose a method of ball-milling sensitizing dyes in organic liquids as a means of spectrally sensitizing silver halide emulsions. Langen et al., in Canadian Patent No. 1,105,761, disclose the use of solid particle milling methods and processes for the introduction of sensitizing dyes and stabilizers in aqueous silver salt emulsions.

Swank and Waack, in U.S. Pat. No. 4,006,025, disclose a process for dispersing sensitizing dyes, wherein said process comprises the steps of mixing the dye particles with water to form a slurry and then milling said slurry at an elevated temperature in the presence of a surfactant to form finely divided particles. Onishi et al., in U.S. Pat. No. 4,474,872, disclose a mechanical grinding method for dispersing certain sensitizing dyes in water without the aid of a dispersing agent or wetting agent. This method relies on pH control in the range of 6-9 and temperature control in the range of 60°-80° C.

Factor and Diehl, in U.S. Pat. No. 4,948,718, disclose solid particle dispersions of dyes for use as filter dyes in photographic elements. They disclose that such dyes can be dispersed as solid particle dispersions by precipitating or reprecipitating (solvent or pH shifting), by ball-milling, by sand-milling, or by colloid-milling in the presence of a dispersing agent.

PROBLEM TO BE SOLVED BY THE  
INVENTION

The crystallization of couplers in amorphous coupler dispersions during storage, during the preparation of photographic elements, and during the storage of photographic elements is a well known deleterious result of the metastability of amorphous coupler dispersions. Such crystallization usually leads to crystallites in excess of 10  $\mu\text{m}$  in largest dimension. Said crystallites cause unwanted scattering of light in photographic elements and loss of gloss, result in substantially decreased specific surface area and decreased effective coupling activity in development processes, and cause gelation of melts and clogging of filters in the coating of photographic elements.

It is known that the preparation of dispersions of couplers and dyes by pH-shifting and by solvent-shifting generally results in said couplers and dyes being in an amorphous physical state, rather than in a crystalline state. Such dispersions are metastable and prone to subsequent crystallization during storage.

Processes utilizing solvent-shifting require the removal of water-miscible solvents subsequent to formation of the dispersion. Such methods for water-miscible solvent removal include evaporation, distillation, and washing. Before and during such solvent removal, the coupler dispersion particles, generally in a metastable thermodynamic state, are prone to ripening and crystallization into large crystallites. Moreover, the utilization of such water-miscible solvents is an unwanted expense.

While it is known that couplers can be dispersed as solid particle dispersions, the practical commercialization of dispersing couplers in photographic film and paper elements has not come to significant fruition be-

cause such dispersions of couplers are generally not reactive enough to provide sufficient image dye densities. In particular, solid particle dispersions of micro-crystalline couplers are particularly inactive in color development solutions when said couplers lack significant solubilization such as imparted by sulfonic acid or carboxyl groups.

It is known that very small-particle, amorphous, and aqueous dispersions of color couplers, as prepared by pH or solvent-shifting, can be combined with aqueous dispersions of permanent solvent to yield improved activity. Said solvent dispersions require a separate process for their formation, whether they are prepared as oil-in-water emulsions or as solvent-loaded latex dispersions. Such separate preparations incur the added cost of surfactant and other dispersing aids, and in many cases the additional cost of said latex. Additional and unwanted costs are incurred in the storage of permanent solvent dispersions.

These and other problems may be overcome by the practice of our invention.

#### SUMMARY OF THE INVENTION

An object of this invention is to provide microcrystalline coupler dispersions with greatly reduced propensity to ripen into coupler crystallites that clog filters and cause unwanted light scattering effects in coated photographic elements. Another object of this invention is to provide microcrystalline coupler dispersions that eliminate the need for water-miscible solvent removal subsequent to particle formation.

A further object of this invention is to greatly reduce the need to prepare permanent solvent dispersions and the costs associated with preparing and storing such dispersions.

These and other objects of the invention are generally accomplished by providing a photographic coupler dispersion comprising colloidal microcrystalline particles of coupler, wherein said particles are wetted with an activating and water-immiscible organic solvent. In another embodiment the invention provides a color photographic element comprising a support bearing at least one photographic silver halide emulsion layer and a microcrystalline coupler dispersion in reactive association with said emulsion layer, wherein said coupler is wetted with an activating water-immiscible organic solvent.

#### BRIEF DESCRIPTION OF THE DRAWINGS

FIG. 1. Sensitometry for coatings of coupler C1, without (curve 1) and with S2 (1:0.25, curve 2; 1:0.5, curve 3), processed in developer A.

FIG. 2. Sensitometry for coatings of coupler C1, without (curve 4) and with S2 (1:0.25, curve 5; 1:0.5, curve 6), processed in developer B.

FIG. 3. Sensitometry for coatings of coupler C2, without (curve 7) and with S2 (1:0.25, curve 8; 1:0.5, curve 9), processed in developer A.

FIG. 4. Sensitometry for coatings of coupler C3, without (curve 10) and with S2 (1:0.25, curve 11; 1:0.5, curve 12), processed in developer A.

FIG. 5. Sensitometry for coatings of coupler C3, without (curve 13) and with S2 (1:0.25, curve 14; 1:0.5, curve 15), processed in developer B.

FIG. 6. Sensitometry for coatings of coupler C4, without (curve 16) and with S2 (1:0.5, curve 17; 1:1, curve 18), processed in developer A.

FIG. 7. Sensitometry for coatings of coupler C5, without (curve 19) and with S2 (1:0.25, curve 20; 1:0.5, curve 21), processed in developer A.

FIG. 8. Sensitometry for coatings of coupler C5, without (curve 22) and with S2 (1:0.25, curve 23; 1:0.5, curve 24), processed in developer B.

FIG. 9. Sensitometry for coatings of coupler M1, without (curve 25) and with S2 (1:0.25, curve 26; 1:0.5, curve 27), processed in developer A.

FIG. 10. Sensitometry for coatings of coupler M1, without (curve 28) and with S2 (1:0.25, curve 29; 1:0.5, curve 30), processed in developer B.

FIG. 11. Sensitometry for coatings of coupler M1, without (curve 31) and with S1 (1:0.25, curve 32; 1:0.5, curve 33), processed in developer A.

FIG. 12. Sensitometry for coatings of coupler M1, without (curve 34) and with S2 (1:0.25, curve 35; 1:0.5, curve 36), processed in developer B.

FIG. 13. Sensitometry for coatings of coupler M2, without (curve 37) and with S2 (1:0.5, curve 38; 1:1, curve 39), processed in developer B.

FIG. 14. Sensitometry for coatings of coupler M3, without (curve 40) and with S2 (1:0.5, curve 41), processed in developer A.

FIG. 15. Sensitometry for coatings of coupler M3, without (curve 42) and with S2 (1:0.5, curve 43), processed in developer B.

FIG. 16. Sensitometry for coatings of coupler M4, without (curve 44) and with S1 and S17 (1:1:0.5, curve 45), processed in developer A.

FIG. 17. Sensitometry for coatings of coupler M4, without (curve 46) and with S1 and S17 (1:1:0.5, curve 47), processed in developer B.

FIG. 18. Sensitometry for coatings of coupler MS, without (curve 48) and with S1 and S17 (1:0.5:0.25, curve 49; 1:1:0.5, curve 50), processed in developer A.

FIG. 19. Sensitometry for coatings of coupler M5, without (curve 51) and with S1 and S17 (1:0.5:0.25, curve 52; 1:1:0.5, curve 53), processed in developer B.

FIG. 20. Sensitometry for coatings of coupler Y1, without (curve 54) and with S2 (1:0.25, curve 55), processed in developer A.

FIG. 21. Sensitometry for coatings of coupler Y1, without (curve 56) and with S2 (1:0.25, curve 57), processed in developer B.

FIG. 22. Sensitometry for coatings of coupler Y2, without (curve 58) and with S2 (1:0.25, curve 59; 1:0.5, curve 60), processed in developer A.

FIG. 23. Sensitometry for coatings of coupler Y2, without (curve 61) and with S2 (1:0.25, curve 62; 1:0.5, curve 63), processed in developer A.

#### ADVANTAGEOUS EFFECT OF THE INVENTION

The microcrystalline coupler dispersions of the present invention greatly reduce the propensity for coupler ripening into large crystallites greater than about 10  $\mu\text{m}$  in average dimension that clog filters, form interconnected gel structures and networks, and cause unwanted light scattering effects in coated photographic elements. The microcrystalline coupler dispersions of the invention provide improved control of reactivity with respect to image dye formation and largely eliminate dispersion reactivity variability due to uncontrolled coupler crystallization.

DETAILED DESCRIPTION OF THE  
INVENTION

The couplers suitable for this invention may be any couplers that can be dispersed as solid particle micro-crystalline dispersions in an aqueous medium. Said couplers are substantially water insoluble at the pH and temperatures of dispersion preparation and use. Typical of such compounds are most photographic color couplers, including those which contain ionizing groups of moderate  $pK_a$  such as carboxyl groups and sulfonamido groups.

The term microcrystalline means that long range order among the coupler molecules exists in the dispersion particles such that a sufficient number of such particles in a scattering-volume element will provide a conventional-looking powder diffraction pattern and d-spacings characteristic of small crystalline particles. Such scattering and diffraction criteria are explained and illustrated by H. P. Klug and L. E. Alexander in *X-ray Diffraction Procedures* (John Wiley & Sons, New York, 1974). Couplers are usually obtained in powdered crystalline form as a natural course of their synthesis and purification. In cases where couplers are obtained in an amorphous form, crystallization can be induced by methods well known in the art, such as thermal annealing, seed crystallization, crystallization from alternative solvents, etc. The expression microcrystalline particles means that said particles are in a physical state as described above in the definition of microcrystalline, and further that said particles are smaller than 5  $\mu\text{m}$  in average dimension.

Typical couplers which form cyan dyes upon reaction with oxidized color developing agents are described in such representative patents as U.S. Pat. Nos. 2,313,586, 2,367,531, 2,369,929, 2,423,730, 2,474,293, 2,772,162, 2,801,171, 2,895,826, 3,002,836, 3,034,892, 3,041,236, 3,419,390, 3,476,563, 3,476,565, 3,772,002, 3,779,763, 3,996,252, 4,124,396, 4,248,962, 4,254,212, 4,282,312, 4,296,199, 4,296,200, 4,327,173, 4,333,999, 4,334,011, 4,427,767, 4,430,423, 4,443,536, 4,444,872,

4,451,559, 4,457,559, 4,500,635, 4,511,647, 4,518,687, 4,526,864, 4,557,999, 4,564,586, 4,565,777, 4,579,813, 4,613,564, 4,690,889, 4,775,616, and 4,874,689, in Canadian Patent No. 625,822, in European Patent Application No. 0 283 938 A1, and in European Patent No. 067 689B1, the disclosures of which are incorporated by reference. Suitable couplers that form cyan dyes upon reaction with oxidized color developing agents are of the phenol type and the naphthol type. Typical couplers which form magenta dyes upon reaction with oxidized color developing agents are described in such representative patents and publications as U.S. Pat. Nos. 1,969,479, 2,311,082, 2,343,703, 2,369,489, 2,600,788, 2,908,573, 3,061,432, 3,062,653, 3,152,896, 3,311,476, 3,419,391, 3,519,429, 3,615,506, 3,725,067, 3,935,015, 3,936,015, 4,119,361, 4,120,723, 4,351,897, 4,385,111, 4,413,054, 4,443,536, 4,500,630, 4,522,916, 4,540,654, 4,581,326, 4,774,172, 4,853,319, and 4,874,689, Japanese Published Patent Application No. 60/170,854, European Patent Publication Nos. 0 170 164, 0 177 765, 0 240 852 A1, 0 283 938 A1, 0 284 239 A1, 0 284 240 A1, and 0 316 955 A3, and *Research Disclosures* 24220 (June 1984) and 24230 (June 1984), the disclosures of which are incorporated by reference. Suitable couplers that form magenta dyes include pyrazolone, pyrazolotriazole, and pyrazolobenzimidazole compounds. Typical couplers which form yellow dyes upon reaction with oxidized color developing agent are described in such representative U.S. Pat. Nos. as 2,298,443, 2,875,057, 2,407,210, 2,875,057, 3,265,506, 3,384,657, 3,408,194, 3,415,652, 3,447,928, 3,542,840, 3,894,875, 3,933,501, 4,022,620, 4,046,575, 4,095,983, 4,133,958, 4,182,630, 4,203,768, 4,221,860, 4,326,024, 4,401,752, 4,443,536, 4,529,691, 4,587,205, 4,587,207 and 4,617,256, 4,622,287, 4,623,616, and in European Patent Applications 0 259 864 A2, 0 296 793 A1, 0 283 938 A1, and 0 316 955 A3, the disclosures of which are incorporated by reference. Suitable yellow dye image forming couplers are acylacetamides, such as benzoylacetanilides and pivaloylacetanilides. Examples of suitable cyan dye-forming couplers include the following:



5,401,623

7

8

-continued

C3



C4



C-5



C6



C7



C8



C9



C10

5,401,623

9

10

-continued



C11



C12



C13



C14



C15



C16



C17

-continued



C18



C19



C20



C21



622



623



C24

-continued



C25



C26

Examples of suitable magenta dye-forming couplers include the following:

25



M1



M2



M3

5,401,623

**15****16**

-continued

**M4****M5****M6****M7****M8**

-continued



M9



M10



M11



M-12



M13

19

5,401,623

20

-continued

M14



M15



M16



M17



M18



M19



-continued



-continued



25

5,401,623

26

-continued

M30



M31



M32



M33



M34



-continued



M35



M36



M37



M38



M39



M40

-continued



M41



M42



M43

Examples of suitable yellow dye-forming couplers include the following:



Y1



Y2

5,401,623

31

32

-continued

Y3



Y4



Y5



Y6



Y7



Y8



-continued



Y9



Y10



Y11



Y12



Y13



Y14

-continued



-continued



Y20



Y21



Y22



Y23



Y24

-continued

Y25



Y26



Preferred couplers for the invention dispersions, photographic elements, and processes for forming dispersions include C1, C2, C3, C4, C5, M1, M2, M3, M4, M5, Y1, and Y2 because of their ready dispersability by roller-milling.

Dispersions of the present invention comprise coupling agents that react with the oxidized product of a primary amine developing agent. Said developing agents are preferably selected from the group comprising 4-amino-N,N-diethylaniline hydrochloride; 4-amino-3-methyl-N,N-diethyl aniline hydrochloride; 4-amino-3-methyl-N-ethyl-N-( $\beta$ -methanesulfonamidoethyl)aniline sulfate hydrate; 4-amino-3-methyl-N-ethyl-N-( $\beta$ -hydroxyethyl)aniline sulfate; 4-amino-3-( $\beta$ -methane sulfonamidoethyl)-N,N-diethylaniline hydrochloride; 4-amino-3-methyl-N-ethyl-N-( $\beta$ -methanesulfonamidoethyl)aniline sesquisulfate monohydrate; and 4-amino-3-methyl-N-ethyl-N-(2-methoxyethyl)aniline di-p-toluenesulfonic acid.

The invention colloidal dispersions of microcrystalline coupler can be obtained by any of the methods for imparting mechanical shear well known in the art, such as those methods described in U.S. Pat. Nos. 2,581,414 and 2,855,156 and in Canadian Patent No. 1,105,761, the disclosures of which are incorporated herein by reference. These methods include solid-particle milling methods such as ball-milling, pebble-milling, roller-milling, sand-milling, bead-milling, dyno-milling, Masap-milling, and media-milling. These methods further include colloid milling, milling in an attriter, dispersing with ultrasonic energy, and high speed agitation (as disclosed by Onishi et al. in U.S. Pat. No. 4,474,872 and incorporated herein by reference). Ball-milling, roller-milling, media-milling, and milling in an attriter are preferred milling methods because of their ease of operation, clean-up, and reproducibility.

Alternatively, coupler dispersions wherein said coupler is present in an amorphous physical state may be prepared by well known methods including colloid milling, homogenization, high speed stirring, sonication methods. The amorphous physical state of said coupler may then be transformed into a microcrystalline physical state by methods including thermal annealing and chemical annealing. Thermal annealing methods in-

30 clude temperature programmed thermal cycling to temperatures above any glass transition temperature of the amorphous coupler. Preferred thermal annealing comprises cycling said dispersion over the temperature 35 range of 17° to 90° C. Said cycling may comprise any sequence of temperature changes that promotes micro-crystalline phase formation from an extant amorphous physical state. Typically the duration of high temperature intervals are chosen to activate said phase formation 40 while minimizing particle growth from ripening and collision processes. Chemical annealing methods include incubation with chemical agents that modify partitioning of couplers and surfactants between the continuous phase of said dispersion and the discontinuous phase. Such agents include hydrocarbons (such as 45 hexadecane), surfactants, alcohols (such as butanol, pentanol, and undecanol), and high boiling organic solvents. Said agents may be added to the dispersion during or subsequent to particle formation. Said chemical annealing 50 may include incubating said dispersion at 17° to 90° C. in the presence of said agent, stirring said dispersion in the presence of said agent, adding said agent and then removing it slowly by diafiltration methods.

55 The formation of colloidal dispersions in aqueous media usually requires the presence of dispersing aids such as surfactants, surface active polymers, and hydrophilic polymers. Such dispersing aids have been disclosed by Chari et al. in U.S. Pat. No. 5,008,179 (columns 13-14) and by Bagchi and Sargeant in U.S. Pat. 60 No. 5,104,776 (see columns 7-13) and are incorporated herein by reference. Preferred dispersing aids include sodium dodecyl sulfate (DA-1), sodium dodecyl benzene sulfonate (DA-2), sodium bis(2-ethyl hexyl)sulfosuccinate (DA-3), Aerosol-22 (Cyanamid), sodium bis(1-methyl pentyl)sulfosuccinate (DA-4), sodium bis(-phenylethyl)sulfosuccinate (DA-5), sodium bis( $\beta$ -phenyl ethyl)sulfosuccinate (DA-6), sodium bis(2-phenyl propyl)sulfosuccinate (DA-7), and the following:



Preferred hydrophilic polymers include gelatin, polyvinylalcohol, and polyvinylpyrrolidone. Such dispersing aids are typically added at level of 1%-200% of dispersed coupler (by weight), and are typically added at preferred levels of 3%-30% of dispersed coupler (by weight).

Colloidal microcrystalline coupler particles less than 1  $\mu\text{m}$  in largest dimension are preferably obtained because of their propensity to scatter less light than larger particles. More preferably because of higher surface to volume ratios, colloidal microcrystalline coupler particles less than 0.2  $\mu\text{m}$  in largest dimension are obtained.

Permanent solvents suitable for use in the present invention may be any water immiscible organic solvent compatible with the microcrystalline couplers utilized. Such solvents have been disclosed, for example, by Bagchi in U.S. Pat. No. 4,970,139 and by Charlet et al. in U.S. Pat. No. 5,008,179, the disclosures of which are incorporated herein by reference. Preferred permanent solvents include tri-cresyl phosphate (S1), di-n-butyl phthalate (S2), N,N-diethyl lauramide (S3), 2,4-di-t-amyl phenol (S4), 2,4-di-n-amyl phenol (S5), N-n-butyl acetanilide (S6), 1,4-cyclohexylene ethylhexanoate (S7),

bis(2-ethylhexyl phthalate (S8), di-n-decyl phthalate (S9), bis(10,11-epoxyundecyl) phthalate (S10), tri-n-hexyl phosphate (S11), dimethyl phthalate (S12), 1-octanol (S13), 1-undecanol (S14), tri-cyclohexyl phosphate (S15), tri-isononyl phosphate (S16), tri-(2-ethylhexyl) phosphate (S17), p-dodecyl phenol (S18), N-n-amyl phthalimide (S19), bis(2-methoxyethyl) phthalate (S20), ethyl-N,N-di-n-butyl carbamate (S21), diethyl phthalate (S22), n-butyl-2-methoxybenzoate (S23), 10 bis(2-n-butoxyethyl) phthalate (S24), diethyl benzylmalonate (S25), guaiacol acetate (S26), tri-m-cresyl phosphate (S26), ethyl phenylacetate (S27), phorone (S28), di-n-butyl sebacate (S29), di-n-octyl phthalate (S30), 15 cresyl diphenyl phosphate (S31), butyl cyclohexyl phthalate (S32), tetrahydrofurfuryl adipate (S33), guaiacol n-caproate (S34), bis(tetrahydrofurfuryl)phthalate (S35), N,N,N',N'-tetraethyl phthalimide (S36), N-n-amyl succinimide (S37), and triethyl citrate (S38).

Permanent solvents can be prepared and initially incorporated into the microcrystalline coupler dispersion by any means well known in the art. Said solvents may initially be prepared as colloidal oil-in-water emulsions, as oil-in-aqueous gelatin emulsions, and as loaded latex dispersions. Such emulsions and loaded latexes may be prepared by well known methods. It is preferred, however, that such solvent incorporation into colloidal dispersions of microcrystalline coupler be done simply and cheaply by pouring the desired amount of permanent solvent directly into the aqueous colloidal dispersion of coupler and agitating with standard means, said means comprising high speed stirring. Interfacial forces dictate the maximum amount of solvent that may be incorporated in this manner, before separate emulsion droplets become kinetically stabilized. The optimal amount of permanent solvent to be added to a given colloidal microcrystalline coupler dispersion will depend on the coupler, the particular crystalline state if polymorphs exist, the particular permanent solvent chosen, and the coupling activity desired in the particular photographic element. Methods of empirically determining such optima are well known to those skilled in the art. Such optima are, however, generally in the preferred coupler to permanent solvent weight ratio range of 1:0.02 to 1:4, and more preferably in the weight ratio range of 1:0.1 to 1:1 in order to minimize solvent loading while obtaining desired coupling activity.

50 In the following discussion of suitable materials for use in the emulsions and elements according to the invention, reference will be made to *Research Disclosure*, December 1989, Item 308119, published by Kenneth Mason Publications Ltd., Emsworth, Hampshire PO10 7DQ, U.K., the disclosures of which are 55 incorporated in their entireties herein by reference. This publication will be identified hereafter as "Research Disclosure".

The support of the element of the invention can be any of a number of well known supports for photographic elements. These include polymeric films, such as cellulose esters (for example, cellulose triacetate and diacetate) and polyesters of dibasic aromatic carboxylic acids with divalent alcohols (such as polyethylene terephthalate), paper, and polymer-coated paper.

55 The photographic elements according to the invention can be coated on the selected supports as described in Research Disclosure Section XVII and the references cited therein.

The radiation-sensitive layer of a photographic element according to the invention can contain any of the known radiation-sensitive materials, such as silver halide, or other light sensitive silver salts. Silver halide is preferred as a radiation-sensitive material. Silver halide emulsions can contain, for example, silver bromide, silver chloride, silver iodide, silver chlorobromide, silver chloroiodide, silver bromoiodide, or mixtures thereof. The emulsions can include coarse, medium, or fine silver halide grains bounded by 100, 111, or 110 crystal planes.

The silver halide emulsions employed in the elements according to the invention can be either negative-working or positive-working. Suitable emulsions and their preparation are described in Research Disclosure Sections I and II and the publications cited therein.

Also useful are tabular grain silver halide emulsions. In general, tabular grain emulsions are those in which greater than 50 percent of the total grain projected area comprises tabular grain silver halide crystals having a grain diameter and thickness selected so that the diameter divided by the mathematical square of the thickness is greater than 25, wherein the diameter and thickness are both measured in microns. An example of tabular grain emulsions is described in U.S. Pat. No. 4,439,520. Suitable vehicles for the emulsion layers and other layers of elements according to the invention are described in Research Disclosure Section IX and the publications cited therein. The radiation-sensitive materials described above can be sensitized to a particular wavelength range of radiation, such as the red, blue, or green portions of the visible spectrum or to other wavelength ranges, such as ultraviolet infrared, X-ray, and the like. Sensitization of silver halide can be accomplished with chemical sensitizers such as gold compounds, iridium compounds, or other group VIII metal compounds, or with spectral sensitizing dyes such as cyanine dyes, merocyanine dyes, or other known spectral sensitizers. Exemplary sensitizers are described in Research Disclosure Section IV and the publications cited therein.

Multicolor photographic elements according to the invention generally comprise a blue-sensitive silver halide layer having a yellow color-forming coupler associated therewith, a green-sensitive layer having a magenta color-forming coupler associated therewith, and a red-sensitive silver halide layer having a cyan color-forming coupler associated therewith. Color photographic elements and color-forming couplers are well-known in the art. The elements according to the invention can include couplers as described in Research Disclosure Section VII, paragraphs D, E, F and G and the publications cited therein. These couplers can be incorporated in the elements and emulsions as described in Research Disclosure Section VII, paragraph C and the publications cited therein.

A photographic element according to the invention, or individual layers thereof, can also include any of a number of other well-known additives and layers. These include, for example, optical brighteners (see Research Disclosure Section V), antifoggants and image stabilizers (see Research Disclosure Section VI), light-absorbing materials such as filter layers of inter-grain absorbers, and light-scattering materials (see Research Disclosure Section VII), gelatin hardeners (see Research Disclosure Section X), oxidized developer scavengers, coating aids and various surfactants, over-coat layers, interlayers, barrier layers and antihalation layers (see Research Disclosure Section VII, paragraph

K), antistatic agents (see Research Disclosure Section XIII), plasticizers and lubricants (see Research Disclosure Section XII), matting agents (see Research Disclosure Section XVI), antistain agents and image dye stabilizers (see Research Disclosure Section VII, paragraphs I and J), development-inhibitor releasing couplers and bleach accelerator-releasing couplers (see Research Disclosure Section VII, paragraph F), development modifiers (see Research Disclosure Section XXI), and other additives and layers known in the art.

Photographic elements according to the invention can be exposed to actinic radiation, typically in the visible region of the spectrum to form a latent image as described in Research Disclosure Section XVIII, and then processed to form a visible dye image as described in Research Disclosure Section XIX. Processing can be any type of known photographic processing, although it is preferably carried out at pH 9 to 14.

A negative image can be developed by using one or more of the aforementioned nucleophiles. A positive image can be developed by first developing with a non-chromogenic developer, then uniformly fogging the element, and then developing by a process employing one or more of the aforementioned nucleophiles.

Development is followed by the conventional steps of bleaching, fixing, or bleach-fixing, to remove silver and silver halide, washing, and drying. Bleaching and fixing can be performed with any of the materials known to be used for that purpose. Bleach baths generally comprise an aqueous solution of an oxidizing agent such as water soluble salts and complexes of iron (III) (such as potassium ferricyanide, ferric chloride, ammonium or potassium salts of ferric ethylenediaminetetra-acetic acid), water-soluble dichromates (such as potassium, sodium, and lithium dichromate), and the like. Fixing baths generally comprise an aqueous solution of compounds that form soluble salts with silver ions, such as sodium thiosulfate, ammonium thiosulfate, potassium thiocyanate, sodium thiocyanate, thioureas, and the like.

## EXAMPLES

### Dispersion Preparation

Solid particle coupler dispersions were prepared by roller milling methods. Typically, a 250-500 mL glass jar containing the charge of coupler, water, dispersing aid, and zirconia (2-mm diameter) media was used; roller milling times of 3 to 5 days were used. The initial charge typically consisted of approximately 5-10 g coupler, 1-3 g dispersing aid, 50-100 g water, and 50-100 mL of zirconia beads. After shaking, 3-6 drops of Anti-foam A (Dow; 50 ppm aqueous suspension) were typically added. In most cases, about 5-10 g of 12.5% (w/w) aqueous gelatin was added to the charge. In certain cases a wetting agent such as isopropanol was also added to the charge. After milling, about 40-80 g of 12.5% aqueous gelatin was added to the jar, and the jar was placed back on the roller mill for a few minutes to achieve good mixing. The dispersion was then filtered to separate the zirconia beads. In cases where permanent solvent was added to the dispersion, an appropriate weight of the permanent solvent was then mixed with an aliquot of the dispersion for about 5 minutes using a Polytron mixer. Dispersions without added permanent solvent were also subjected to about 5 minutes of mixing with a Polytron mixer.

## Coating and Evaluation

Experimental coatings were prepared of each dispersion in a two-layer test format coated on transparent film support. The first layer typically contained about  $1.07 \times 10^{-3}$  (couplers M1, M2, M4, and M5) or  $2.14 \times 10^{-3}$  (couplers C1-C5, M3, Y1, and Y2) mol coupler/m<sup>2</sup>, a polydisperse sulfur and gold sensitized silver bromoiodide emulsion at a level of about  $1.1 \times 10^{-2}$  mol/m<sup>2</sup> as silver, and about 3.76 g/m<sup>2</sup> of gelatin. A second layer containing about 1.07 g/m<sup>2</sup> of gelatin was coated over the first layer. Hardener (1,1'-[oxybis{methylene sulfonyl}]bisethene) was coated at a level corresponding to about 1.5% (w/w) of the total gelatin coated. After coating and chopping, the sensitized strips were exposed on a sensitometer to a tungsten light source though a 0 to 6 density 21-step tablet and processed at 100° F. in one of two developer solutions.

| Developer solution A comprised:                             |              |
|-------------------------------------------------------------|--------------|
| Anhydrous potassium carbonate                               | 37.5 g       |
| Anhydrous sodium sulfate                                    | 4.0 g        |
| Potassium iodide                                            | 1.2 mg       |
| Sodium bromide                                              | 1.3 g        |
| 1,3-Diamino-2-propanoltetraacetic acid                      | 2.5 g        |
| Hydroxylamine sulfate                                       | 2.0 g        |
| KODAK color developing agent CD-4                           | 4.5 g        |
| Water to make 1 liter                                       |              |
| pH @ 27° C.                                                 | 10.00 ± 0.03 |
| Developer solution B comprised:                             |              |
| Triethanolamine                                             | 9.89 g       |
| Phorwite REU (Mobay)                                        | 0.80 g       |
| Benzyl alcohol                                              | 15.05 g      |
| Hydroxylamine sulfate                                       | 3.20 g       |
| Lithium chloride                                            | 1.68 g       |
| Lithium polystyrenesulfonate (30% aqueous solution)         | 0.20 g       |
| KODAK color developing agent CD-3                           | 5.20 g       |
| Potassium sulfite (45% aqueous solution)                    | 4.19 g       |
| 1-Hydroxyethyl-1,1-diphosphonic acid (60% aqueous solution) | 0.93 g       |
| Anhydrous potassium carbonate                               | 29.62 g      |
| Potassium bromide                                           | 0.60 g       |
| Potassium chloride                                          | 0.50 g       |
| Potassium hydroxide (45% aqueous solution)                  | 0.92 g       |
| Water to make 1 liter                                       |              |
| pH @ 27° C.                                                 | 10.00 ± 0.03 |

After development for 1 minute, the strips were, with nitrogen burst agitation, immersed in a stop bath for 1 minute, rinsed in water for 3 minutes, immersed in an iron(III) bleach solution for 3 minutes, rinsed in water for 3 minutes, immersed in a thiosulfate-based fixing solution for 3 minutes, rinsed in water for 3 minutes, and dried. Sensitometric curves were recorded through status-M filters.

## Examples 1-6

Roller milled dispersions of coupler C1 were prepared by combining 10 g of C1, 2.5 g Aerosol-OT, about 110 g water, 10 g 12.5% (w/w) aqueous gelatin 3.5 g isopropanol, 50 mL zirconia beads (about 1.8 mm in diameter), and about 6 drops of Anti-foam A. This mixture was milled for 5 days, and then about 70 g of melted 12.5% aqueous gelatin was added with mixing. The resulting dispersion was filtered, chill set, and stored in the cold until used.

Modified dispersions containing the permanent solvent di-n-butyl phthalate (S2) at C1:S2 weight ratios of 1:0.25 and 1:0.5 were prepared by adding an appropriate

amount of S2 to the permanent solvent free dispersion and mixing in a Polytron stirrer for about 5 min. Electron micrographs of these dispersions showed platelike morphology with aspect ratios in the range of 20-60 and with effective circular diameters in the range of 1-4  $\mu\text{m}$ .

Sensitometry for test coatings of these dispersions after processing in developer A is illustrated in FIG. 1 for Examples 1-3 (curves 1-3, respectively) for the dispersion without added permanent solvent (curve 1), the dispersion 1:0.25 in C1:S2 ratio (curve 2), and the dispersion 1:0.5 in C1:S2 ratio (curve 3). These curves show that a large latitude in apparent dye-forming activity is available by varying the amount of added permanent solvent. Similar results, although highlighted in the upper scale, are illustrated in FIG. 2 for Examples 4-6 (curves 4-6, respectively) for these same test coatings processed in developer B, where the dispersion without added permanent solvent corresponds to curve 4, the dispersion 1:0.25 in C1:S2 ratio corresponds to curve 5, and the dispersion 1:0.5 in C1:S2 ratio corresponds to curve 6.

## Examples 7-9

Three roller milled dispersions of coupler C2 were prepared by combining 5 g of C2, 1 g Alkanol-XC, about 50 g water, 5 g melted 12.5% (w/w) aqueous gelatin, 100 mL zirconia beads, and about 4 drops of Anti-foam A in triplicate. These mixtures were milled for 3 days, filtered, and then combined into a single sample (155 g yield). About 102 g of melted 12.5% aqueous gelatin was added with mixing. The resulting dispersion was then chill set, and stored in the cold until used.

Modified dispersions containing the permanent solvent di-n-butyl phthalate (S2) at C2:S2 weight ratios of 1:0.5 and 1:1 were prepared by adding an appropriate amount of S2 to the permanent solvent-free dispersion and mixing in a Polytron stirrer for about 5 min. Electron micrographs of these dispersions showed polydisperse platelike morphology. Dispersions with added S2 showed no significant morphological dissimilarity to the dispersion prepared without added S2.

Sensitometry for test coatings of these dispersions after processing in developer A is illustrated in FIG. 3 for Examples 7-9 (curves 7-9, respectively) for the dispersion without added permanent solvent (curve 7), the dispersion 1:0.5 in C2:S2 ratio (curve 8), and the dispersion 1:1 in C2:S2 ratio (curve 9). These curves also show that a large latitude in apparent dye-forming activity is available by varying the amount of added permanent solvent.

## Examples 10-15

Roller milled dispersions of coupler C3 were prepared by combining about 10 g of C3, 2.5 g Aerosol-OT, about 110 g water, 10 g of melted 12.5% (w/w) aqueous gelatin, 3.5 g isopropanol, 50 mL zirconia beads, and about 6 drops of Anti-foam A. This mixture was milled for 5 days, and then about 70 g of melted 12.5% aqueous gelatin was added with mixing. The resulting dispersion was filtered, chill set, and stored in the cold until used.

Modified dispersions containing the permanent solvent di-n-butyl phthalate (S2) at C3:S2 weight ratios of 1:0.25 and 1:0.5 were prepared by adding an appropriate amount of S2 to aliquots of the permanent solvent free dispersion and mixing in a Polytron stirrer for about 5

min. Electron micrographs of these dispersions showed that three-dimensional parallelepiped morphology predominates for this method of preparation. Microcrystalline particle sizes were polydisperse, and in the range of approximately 0.1–1  $\mu\text{m}$ .

Sensitometry for test coatings of these dispersions after processing in developer A is illustrated in FIG. 4 for Examples 10–12 (curves 10–12, respectively) for the dispersion without added permanent solvent (curve 10), the dispersion 1:0.25 in C3:S2 ratio (curve 11), and the dispersion 1:0.5 in C3:S2 ratio (curve 12). These curves again show that a large latitude in apparent dye-forming activity is available by varying the amount of added permanent solvent. Similar results are illustrated in FIG. 5 for Examples 13–16 (curves 13–15, respectively) for these same test coatings processed in developer B, where the dispersion without added permanent solvent corresponds to curve 13, the dispersion 1:0.25 in C3:S2 ratio corresponds to curve 14, and the dispersion 1:0.5 in C3:S2 ratio corresponds to curve 15.

#### Examples 16–18

Roller milled dispersions of coupler C4 were prepared by combining about 10 g of C4, 10 g 10% aqueous Olin-10G, 10 g 6.8% aqueous TX-200, about 208 g water, 20 g isopropanol, and about 130 mL zirconia beads. This mixture was milled for 5 days, and then about 80 g of melted 12.5% aqueous gelatin was added with mixing. The resulting dispersion was filtered, chill set, and stored in the cold until used.

Modified dispersions containing the permanent solvent di-n-butyl phthalate (S2) at C4:S2 weight ratios of 1:0.5 and 1:1 were prepared by adding an appropriate amount of S2 to aliquots of the permanent solvent free dispersion and mixing in a Polytron stirrer for about 5 min. Electron micrographs of these dispersions showed that rectangular plates predominated in the particle morphology and that the larger particles exhibited aspect ratios on the order of 10. Particle sizes were polydisperse, and many of the particles were greater than 2  $\mu\text{m}$  in length, with widths running about 20–25% of the lengths. The average equivalent circular diameter was about 0.5  $\mu\text{m}$ .

Sensitometry for test coatings of these dispersions after processing in developer A is illustrated in FIG. 6 for Examples 16–18 (curves 16–18, respectively) for the dispersion without added permanent solvent (curve 16), the dispersion 1:0.5 in C4:S2 ratio (curve 17), and the dispersion 1:1 in C4:S2 ratio (curve 18). The effects of added permanent solvent are particularly evident in the upper scale.

#### Examples 19–24

Roller milled dispersions of coupler C5 were prepared by combining about 25 g of C5, about 6.3 g of 55 Aerosol-OT, about 250 g water, about 25 g melted 12.5% aqueous gelatin, and about 500 mL zirconia beads. This mixture was milled for 5 days, warmed to about 40° C., and then about 175 g of melted 12.5% aqueous gelatin was added with mixing. The resulting dispersion was filtered, chill set, and stored in the cold until used.

Modified dispersions containing the permanent solvent di-n-butyl phthalate (S2) at C5:S2 weight ratios of 1:0.25 and 1:0.5 were prepared by adding an appropriate amount of S2 to aliquots of the permanent solvent free dispersion and mixing in a Polytron stirrer for about 5 min. Electron micrographs of these dispersions showed

that the predominant particle morphology was plate-like, and that the morphology in the dispersions with added S2 was identical to that without.

Sensitometry for test coatings of these dispersions after processing in developer A is illustrated in FIG. 7 for Examples 19–21 (curves 19–21, respectively) for the dispersion without added permanent solvent (curve 19), the dispersion 1:0.25 in C5:S2 ratio (curve 20), and the dispersion 1:0.5 in C5:S2 ratio (curve 21). The effects of added permanent solvent are evident throughout the illustrated scale. Similar results are illustrated in FIG. 8 for Examples 22–24 (curves 22–24, respectively) for these same test coatings processed in developer B, where the dispersion without added permanent solvent corresponds to curve 22, the dispersion 1:0.25 in C5:S2 ratio corresponds to curve 23, and the dispersion 1:0.5 in C5:S2 ratio corresponds to curve 24. Here the effects of added permanent solvent are most evident in the upper scale.

20

#### Examples 25–36

Three roller milled dispersions of coupler M1 were prepared by combining 5 g of M1, 1 g Alkanol-XC, about 50 g water, 5 g melted 12.5% (w/w) aqueous gelatin, 100 mL zirconia beads, and about 4 drops of Anti-foam A in triplicate. These mixtures were milled for 3 days, warmed to 45° C., filtered, and then combined into a single sample (159 g yield). About 104 g of melted 12.5% aqueous gelatin was added with mixing. 25 The resulting dispersion was then chill set, and stored in the cold until used.

Modified dispersions containing the permanent solvent di-n-butyl phthalate (S2) at M1:S2 weight ratios of 1:0.25 and 1:0.5 were prepared by adding an appropriate 35 amount of S2 to aliquots of the permanent solvent-free dispersion and mixing in a Polytron stirrer for about 5 min. Electron micrographs of these dispersions showed polydisperse irregularly shaped particles with sizes in the range of 0.2–0.6  $\mu\text{m}$ . Added S2 appeared to smooth 40 some of the surface irregularities.

Sensitometry for test coatings of these dispersions after processing in developer A is illustrated in FIG. 9 for Examples 25–27 (curves 25–27, respectively) for the dispersion without added permanent solvent (curve 25), the dispersion 1:0.25 in M1:S2 ratio (curve 26), and the dispersion 1:0.5 in M1:S2 ratio (curve 27). The effects of added permanent solvent appear identical for the 1:0.25 and 1:0.5 M1:S2 ratios. Similar results are illustrated in FIG. 10 for Examples 28–30 (curves 28–30, respectively) for these same test coatings processed in developer B, where the dispersion without added permanent solvent corresponds to curve 28, the dispersion 1:0.25 in M1:S2 ratio corresponds to curve 29, and the dispersion 1:0.5 in M1:S2 ratio corresponds to curve 30.

Modified dispersions containing the permanent solvent tri-cresyl phosphate (S1) at M1:S1 weight ratios of 1:0.25 and 1:0.5 were prepared by adding an appropriate amount of S1 to aliquots of the permanent solvent-free dispersion and mixing in a Polytron stirrer for about 5 min. Electron micrographs of these dispersions showed polydisperse irregularly shaped particles with sizes in the range of 0.2–0.6  $\mu\text{m}$ . Added S1 appeared not to affect this surface roughness.

Sensitometry for test coatings of these dispersions after processing in developer A is illustrated in FIG. 11 for Examples 31–33 (curves 31–33, respectively) for the dispersion without added permanent solvent (curve 31), the dispersion 1:0.25 in M1:S1 ratio (curve 32), and the

dispersion 1:0.5 in M1:S1 ratio (curve 33). The effects of added permanent solvent appear nearly identical for the 1:0.25 and 1:0.5 M1:S1 ratios. Similar results are illustrated in FIG. 12 for Examples 34-36 (curves 34-36, respectively) for these same test coatings processed in developer B, where the dispersion without added permanent solvent corresponds to curve 34, the dispersion 1:0.25 in M1:S1 ratio corresponds to curve 35, and the dispersion 1:0.5 in M1:S1 ratio corresponds to curve 36.

#### Examples 37-39

Roller milled dispersions of coupler M2 were prepared by combining about 4.5 g of M2, about 2 g 10% aqueous Olin-10G, about 4 g 6.8% aqueous TX-200, about 6 g isopropanol, about 32 g water, and about 65 mL zirconia beads. This mixture was milled for 5 days, and then about 36 g of melted 12.5% aqueous gelatin was added with mixing, followed by 15 min of sonication with an ultrasonic probe. The resulting dispersion was filtered, chill set, and stored in the cold until used.

Modified dispersions containing the permanent solvent di-n-butyl phthalate (S2) at M2:S2 weight ratios of 1:0.5 and 1:1 were prepared by adding an appropriate amount of S2 to aliquots of the permanent solvent free dispersion and mixing in a Polytron stirrer for about 5 min. Electron micrographs of these dispersions showed a bimorphic population of particles. There was a small population of rods about 0.02  $\mu\text{m}$  in diameter and about 0.5-1.0  $\mu\text{m}$  in length. The predominant morphology was plate-like and polydisperse in shape, size, and aspect ratio. The predominant shape was rectangular with widths ranging from 0.1-0.5  $\mu\text{m}$  and lengths ranging from 0.1-2  $\mu\text{m}$ . There was no obvious effect of the added permanent solvent S2 on the plate-like particles in the 1:0.5 (M2:S2) modified dispersion, although very few of the small rods were evident. The 1:1 modified dispersion showed more of a ripening effect of the added solvent. Some of the smaller plates appeared to have been transformed into three-dimensional particles.

Sensitometry for test coatings of these dispersions after processing in developer B is illustrated in FIG. 13 for Examples 37-39 (curves 37-39, respectively) for the dispersion without added permanent solvent (curve 37), the dispersion 1:0.5 in M2:S2 ratio (curve 38), and the dispersion 1:1 in M2:S2 ratio (curve 39). The effects of added permanent solvent are evident in the upper scale.

#### Examples 40-43

A roller milled dispersion of coupler M3 was prepared by combining 5 g of M3, 1 g Alkanol-XC, about 50 g water, 5 g melted 12.5% (w/w) aqueous gelatin, 100 mL zirconia beads, and about 4 drops of Anti-foam A, and milling for 3 days. After milling the dispersion was warmed to 40° C. and then combined with about 40 g of melted 12.5% aqueous gelatin with mixing. The resulting dispersion was then filtered, chill set, and stored in the cold until used.

A modified dispersion containing the permanent solvent di-n-butyl phthalate (S2) at a M3:S2 weight ratio of 1:0.5 was prepared by adding an appropriate amount of S2 to an aliquot of the permanent solvent-free dispersion and mixing in a Polytron stirrer for about 5 min. Electron micrographs of these dispersions showed that the dispersion without added S2 was bimorphic and comprised a population of polydisperse irregularly shaped platelike particles with equivalent circular diameters in the range of 0.2-0.8  $\mu\text{m}$  and aspect ratios in the range of 4-6 and another population comprising 0.02

$\mu\text{m}$  diameter rods about 0.2  $\mu\text{m}$  in length. Added S2 did not appear to modify the morphology of the large particles but did appear to convert the small rods into small sphere approximately 0.06  $\mu\text{m}$  in diameter.

Sensitometry for test coatings of these dispersions after processing in developer A is illustrated in FIG. 14 for Examples 40 and 41 (curves 40 and 41, respectively) for the dispersion without added permanent solvent (curve 40) and the dispersion 1:0.5 in M3:S2 ratio (curve 41). Added permanent solvent dramatically increases the coupling activity. Similar results are illustrated in FIG. 15 for Examples 42 and 43 (curves 42 and 43, respectively) for these same test coatings processed in developer B, where the dispersion without added permanent solvent corresponds to curve 42, and the dispersion 1:0.5 in M3:S2 ratio corresponds to curve 43. The effects of added solvent in this case are more significant in the upper scale.

#### Examples 44-47

A roller milled dispersion of coupler M4 was prepared by combining 6 g of M4, 1.2 g Alkanol-XC, about 60 g water, 6 g melted 12.5% (w/w) aqueous gelatin, and about 120 mL zirconia beads. This charge was milled for 3 days. After milling the dispersion was warmed to 45° C. and then combined with about 46.8 g of melted 12.5% aqueous gelatin with mixing. The resulting dispersion was then filtered, chill set, and stored in the cold until used.

A modified dispersion containing the permanent solvents di-n-butyl phthalate (S1) and tri-(2-ethylhexyl) phosphate (S17) at a M4:S2:S17 weight ratio of 1:1:0.5 was prepared by adding appropriate amounts of S2 and S17 to an aliquot of the permanent solvent-free dispersion and mixing in a Polytron stirrer for about 5 min. Electron micrographs of these dispersions showed that the dispersion without added permanent solvent comprised polydisperse irregularly shaped two-dimensional plates 0.2-0.8  $\mu\text{m}$  in equivalent circular diameter. The morphology of the particles in the modified dispersion could not be identified because of the large amount of permanent solvent in the dispersion.

Sensitometry for test coatings of these dispersions after processing in developer A is illustrated in FIG. 16 for Examples 44 and 45 (curves 44 and 45, respectively) for the dispersion without added permanent solvent (curve 44) and the dispersion 1:1:0.5 in M4:S2:S17 ratio (curve 45). Added permanent solvent dramatically increases the coupling activity. Similar results are illustrated in FIG. 17 for Examples 46 and 47 (curves 46 and 47, respectively) for these same test coatings processed in developer B, where the dispersion without added permanent solvent corresponds to curve 46, and the dispersion 1:1:0.5 in M4:S2:S17 ratio corresponds to curve 47. The effects of added solvent in this case are again more significant in the upper scale.

#### Examples 48-53

A roller milled dispersion of coupler M5 was prepared by combining 6 g of M5, 1.2 g Alkanol-XC, about 60 g water, 6 g melted 12.5% (w/w) aqueous gelatin, and about 120 mL zirconia beads. This charge was milled for 3 days. After milling the dispersion was warmed to 45° C. and then combined with about 46.8 g of melted 12.5% aqueous gelatin with mixing. The resulting dispersion was then filtered, chill set, and stored in the cold until used.

Modified dispersions containing the permanent solvents di-n-butyl phthalate (S1) and tri-(2-ethylhexyl) phosphate S17 at M5:S2:S17 weight ratios of 1:0.5:0.25 and 1:1:0.5 were prepared by adding appropriate amounts of S2 and S17 to aliquots of the permanent solvent-free dispersion and mixing in a Polytron stirrer for about 5 min. Electron micrographs of these dispersions showed that the dispersion without added permanent solvent comprised irregularly shaped plates with rough surfaces and equivalent circular diameters in the range of 0.3–0.9  $\mu\text{m}$  in equivalent circular diameter. The morphology of the particles in the modified dispersions was transformed to a more rectangular shape with smoother surfaces.

Sensitometry for test coatings of these dispersions after processing in developer A is illustrated in FIG. 18 for Examples 48–50 (curves 48–50, respectively) for the dispersion without added permanent solvent (curve 48), the dispersion 1:0.5:0.25 in M5:S2:S17 ratio (curve 49), and the dispersion 1:1:0.5 in M5:S2:S17 ratio (curve 50). Added permanent solvent dramatically increases the coupling activity. Similar results are illustrated in FIG. 19 for Examples 51–53 (curves 51–53, respectively) for these same test coatings processed in developer B, where the dispersion without added permanent solvent corresponds to curve 51, the dispersion 1:0.5:0.25 in M5:S2:S17 ratio (curve 52), and the dispersion 1:1:0.5 in M5:S2:S17 ratio corresponds to curve 53. The effects of added solvent in this case are again more significant in the upper scale.

#### Examples 54–57

A roller milled dispersion of coupler Y1 was prepared by combining 10 g of Y1, 2.5 g Aerosol-OT, about 110 g water, 10 g melted 12.5% (w/w) aqueous gelatin, 3.5 g isopropanol, about 50 mL zirconia beads, and about 6 drops of Anti-foam A. This charge was milled for 5 days. After milling the dispersion was combined with about 70 g of melted 12.5% aqueous gelatin with mixing. The resulting dispersion was then filtered, chill set, and stored in the cold until used.

A modified dispersion containing the permanent solvent di-n-butyl phthalate (S2) at a Y1:S2 weight ratio of 1:0.25 was prepared by adding appropriate amounts of S2 to an aliquot of the permanent solvent-free dispersion and mixing in a Polytron stirrer for about 5 min. Electron micrographs of these dispersions showed that the dispersion without added permanent solvent was polydisperse. There was a large population of fines (less than 0.2  $\mu\text{m}$  in diameter) and there was a considerable volume fraction of large (0.2–0.8  $\mu\text{m}$  equivalent circular diameter) plates. The addition of S2 did not appear to modify these morphological features.

Sensitometry for test coatings of these dispersions after processing in developer A is illustrated in FIG. 20 for Examples 54 and 55 (curves 54 and 55, respectively) for the dispersion without added permanent solvent (curve 54) and the dispersion 1:0.25 in Y1:S2 ratio (curve 55). Added permanent solvent dramatically increases the coupling activity. Similar results are illustrated in FIG. 21 for Examples 56 and 57 (curves 56 and 57, respectively) for these same test coatings processed in developer B, where the dispersion without added permanent solvent corresponds to curve 56, and the dispersion 1:0.25 in Y1:S2 ratio corresponds to curve 57. The effects of added solvent in this case are significantly more evident.

#### Examples 58–63

Three roller milled dispersions of coupler Y2 were prepared by combining 5 g of Y2, 1 g Alkanol-XC, about 50 g water, 5 g melted 12.5% (w/w) aqueous gelatin, 100 mL zirconia beads, and about 4 drops of Anti-foam A in triplicate. These mixtures were milled for 3 days, filtered, and then combined into a single sample (165 g yield). About 108 g of melted 12.5% aqueous gelatin was added with mixing. The resulting dispersion was then chill set, and stored in the cold until used.

Modified dispersions containing the permanent solvent di-n-butyl phthalate (S2) at Y2:S2 weight ratios of 1:0.25 and 1:0.5 were prepared by adding an appropriate amount of S2 to the permanent solvent-free dispersion and mixing in a Polytron stirrer for about 5 min. Electron micrographs of the dispersion without added permanent solvent showed that the largest population of particles was about 0.1  $\mu\text{m}$  or less in equivalent spherical diameter. There also was a population of larger plates with rough surfaces of 0.2–0.6  $\mu\text{m}$  in equivalent circular diameter. The addition of S2 apparently facilitated ripening of these particles. Surfaces appeared smoother and an intermediate sized population of plates (0.2  $\mu\text{m}$  equivalent circular diameter) was present.

Sensitometry for test coatings of these dispersions after processing in developer A is illustrated in FIG. 22 for Examples 58–60 (curves 58–60, respectively) for the dispersion without added permanent solvent (curve 58), the dispersion 1:0.25 in Y2:S2 ratio (curve 59), and the dispersion 1:0.5 in Y2:S2 ratio (curve 60). These curves also show that added S2 dramatically increases coupling activity. Similar results are illustrated in FIG. 23 for Examples 61–63 (curves 61–63, respectively) for these same test coatings processed in developer B, where the dispersion without added permanent solvent corresponds to curve 61, the dispersion 1:0.25 in Y2:S2 ratio corresponds to curve 62, and the dispersion 1:0.5 in Y2:S2 ratio corresponds to curve 63.

The invention has been described in detail with particular reference to preferred embodiments thereof, but it will be understood that variations and modifications can be effected within the spirit and scope of the invention.

#### What is claimed is:

1. A photographic coupler dispersion comprising colloidal microcrystalline particles of coupler smaller than 5  $\mu\text{m}$  in average dimension, wherein said particles are wetted with an activating and water-immiscible organic solvent.
2. A dispersion as in claim 1 wherein said particles are less than 1  $\mu\text{m}$  in largest dimension.
3. A dispersion as in claim 2 wherein said particles are less than 0.2  $\mu\text{m}$  in largest dimension.
4. A dispersion as in claim 1 which further comprises a hydrophilic polymer.
5. A dispersion as in claim 4 wherein said polymer is selected from the group comprising gelatin, polyvinyl alcohol, polyvinylpyrrolidone.
6. A dispersion as in claim 1 wherein said coupler reacts with the oxidized product of a primary amine developing agent.
7. A dispersion as in claim 6 wherein said developing agent is selected from the group consisting of 4-amino-N,N-diethylaniline hydrochloride; 4-amino-3-methyl-N,N-diethyl aniline hydrochloride; 4-amino-3-methyl-N-ethyl-N-( $\beta$ -methanesulfonamidoethyl)aniline sulfate

hydrate; 4-amino-3-methyl-N-ethyl-N-( $\beta$ -hydroxyethyl)aniline sulfate; 4-amino-3-( $\beta$ -methanesulfonamido)ethyl-N,N-diethylaniline hydrochloride; 4-amino-3-methyl-N-ethyl-N-( $\beta$ -methanesulfonamidoethyl)aniline sesquisulfate monohydrate; and 4-amino-3-methyl-N-ethyl-N-(2-methoxyethyl)aniline di-p-toluenesulfonic acid.

8. A dispersion as in claim 1 wherein said solvent is selected from the group consisting of tri-cresyl phosphate, di-n-butyl phthalate, N,N-diethyl lauramide, 2,4-di-t-amyl phenol, 2,4-di-n-amyl phenol, N-n-butyl acetanilide, 1,4-cyclohexylene ethylhexanoate, bis(2-ethylhexyl phthalate, di-n-decyl phthalate, bis(10,11-epoxyundecyl) phthalate, tri-n-hexyl phosphate, dimethyl phthalate, 1-octanol, 1-undecanol, tri-cyclohexyl phosphate, tri-isonyl phosphate, tri-92-ethylhexyl) phosphate, p-dodecyl phenol, N-n-amyl phthalimide, bis(2-methoxyethyl) phthalate, ethyl-N,N-di-n-butyl carbamate, diethyl phthalate, n-butyl-2-methoxybenzoate, bis(2-n-butoxyethyl) phthalate, diethyl benzylmalonate, guaiacol acetate, tri-m-cresyl phosphate, ethyl phenylacetate, phorone, di-n-butyl sebacate, di-n-octyl phthalate, cresyl diphenyl phosphate, butyl cyclohexyl phthalate, tetrahydrofurfuryl adipate, guaiacol n-caproate, bis(tetrahydrofurfuryl)phthalate, N,N,N',N'-tetraethyl phthalimide, N-n-amyl succinimide, and triethyl citrate.

9. A dispersion as in claim 1 wherein said solvent is added at a coupler to permanent solvent weight ratio in the range of 1:0.02 to 1:4.

10. A dispersion as in claim 9 wherein said solvent is added at a coupler to permanent solvent weight ratio in the range of 1:0.1 to 1:1.

11. A dispersion as in claim 1 wherein said microcrystalline coupler dispersion is prepared with a dispersing aid.

12. A dispersion as in claim 11 wherein said microcrystalline coupler dispersion is prepared with a dispersing aid selected from the group consisting of sodium dodecyl sulfate, sodium dodecyl benzene sulfonate, sodium bis(2-ethyl hexyl)sulfosuccinate, sodium bis(1-methyl pentyl)sulfosuccinate, sodium bis(phenylethyl)sulfosuccinate, sodium bis( $\beta$ -phenyl ethyl)sulfosuccinate, sodium bis(2-phenyl propyl)sulfosuccinate, and the following:



13. A dispersion as in claim 11 wherein said dispersing aid is present in said dispersion at a coupler to dispersing aid weight ratio of 1:0.01 to 1:2.

14. A dispersion as in claim 13 wherein said dispersing aid is present in said dispersion at a coupler to dispersing aid weight ratio of 1:0.03 to 1:0.3.

15. A color photographic element comprising a support bearing at least one photographic silver halide emulsion layer and a microcrystalline coupler dispersion in reactive association with said emulsion layer, wherein said coupler dispersion comprises microcrystalline particles of coupler smaller than 5  $\mu\text{m}$  in average dimension wetted with an activating water-immiscible organic solvent.

\* \* \* \* \*